

## UNITED STATES PATENT OFFICE

2,039,989

## SULPHONATION OF OILS AND GREASES

Alexander Gressner, Habana, Cuba

No Drawing. Application May 29, 1934,  
Serial No. 728,183

5 Claims. (Cl. 87—12)

This invention relates to the sulphonation of oils and greases (either aliphatic or aromatic oils, saturated or non-saturated oils and greases, as well as their ethers and esters, especially of the glycerylic group of drying, semi-drying or permanent oils or fats with high or medium iodine number, as, e. g., the oils and fats of fluvial-, lacustrine-, or marine-animal origin, with or without the presence of non-saponifiable substances) for use as lubricators, softeners, sizings, mordants, color enhancers, etc. in the textile, tanning and dyeing industries as, e. g. fibre spinneries, weaveries, leather tanning and conditioning plants, etc.

My process allows the sulphonation of organic products (mentioned above) for the purpose of converting said organic substances into emulsive, dispersive, and miscible compounds of high stability, which may be readily incorporated with fluids and solvents as generally applied in the corresponding trades, as, e. g., water, alcohol of various strengths, etc.

According to my process, said organic products (more especially the fatty acids, their ethers and esters, and chiefly the drying semi-drying and permanent oils or fats of animals having a fluvial, lacustrine, marine, or land habitat, also those of vegetable origin, with high or medium molecular weight), acquire emulsive, dispersive, miscive and solutive properties with which may be prepared solutions, suspensions, dispersions or emulsions with or without hydrocarbons or organic products having an acid, neutral, or basic reaction, as of mineral, vegetable or animal oils and fats. The hydrocarbons which I may use and incorporate into any oil or grease sulphonated according to my process are: all aliphatic saturated hydrocarbons (homologues of methane, hexane, heptane, etc.); also all aliphatic non-saturated hydrocarbons (homologues of ethylene, propylene, etc.); also all aromatic hydrocarbons, as f. i. benzene and its homologues, naphthalene, anthracene, etc.; also all naphthenes or cycloparaffines (homologues of trimethylene, heptamethylene, hexanaphthene, etc.).

My process consists in sulphonating one or several of the aforementioned oils or fats, either alone or in the presence of mineral oils or greases, with from ten to fifty percent, or greater percentage, of sulphuric acid, with or without the aid of fuming sulphuric acid. The sulphonation is performed in the presence of one or more acid sulphates of the alkaline metal group, as, for example, acid potassium sulphate ( $KHSO_4$ ). The catalytic action of the group mentioned greatly accelerates the sulphonic reaction and considera-

bly augments the quantity of organically combined sulphuric acid as compared with previous processes, in which as much as 85% of the sulphuric acid employed does not enter into the reaction. The sulphuric acid is either poured all at once, or in a properly graduated stream, into the substance to be sulphonated, according to the cooling capacity of the vat, in order to avoid a sudden and excessive rise of temperature which would result in diminishing the commercial value of the product. After all the acid has been poured into the sulphonating cooling vat, stirring is continued from thirty to sixty minutes longer, during which time the reaction will be thoroughly completed. Immediately afterwards is added any hydrocarbon or hydrocarbons which it is desired to embody in the compound for the purpose of forming an emulsion, dispersion or solution; while this mixture is being cooled down and briskly stirred, the excess sulphuric acid is eliminated to the desired point, preferably to the point where the pH value is between 7 and 9, as I have discovered that neutralization to this value gives to my product its improved emulsive, solutive and dispersive properties. It will be noted that the excess sulphuric acid is neutralized after the addition of the hydrocarbon and not before. This is a feature of my invention, the presence of the sulphuric acid allowing the sulphonated oil and the hydrocarbon to combine into a homogeneous and transparent mixture. Any one of the currently used alkalies will do, as, e. g., hydroxides of soda or potash, carbonates, bicarbonates, gaseous or liquid ammonia, amines, etc. The product may however be made acid, neutral or basic, according to the purpose for which it is to be used. The resulting substance is a clear viscous fluid. Mixed with water or with other solvent, it will go into solution and yield snow-white emulsions of very high stability which will keep unaltered during many weeks.

Typical examples of sulphonation according to my process are given below.

1. Incorporate, under the effects of a powerful and rapidly moving mechanical agitator or mixer, five parts of completely dried and finely pulverized acid sulphate of potash into one hundred parts of sardine oil, or any similar oil, cooled with ice or any other suitable means to  $+10^{\circ} C$ . After thorough incorporation of this catalyst, sulphonation is brought about by adding twenty parts of concentrated sulphuric acid, one half of which, i. e., ten parts, can be poured at once into the vat. Due to the cooling and agitation, the temperature will not rise above  $30^{\circ} C$ . if no more than said ten parts of sulphuric acid were added at

once. Under continued stirring, and if the cooling is properly conducted, the temperature of the mixture will have descended again to the initial 10° C. within 20 minutes from the moment the 5 first ten parts of sulphuric acid were added. At this time, the remaining ten parts of sulphuric acid can be added, either at once, or in a thick stream. The cooling and agitation are to be continued for an hour from the time the sulphonating process was started. One hour is enough 10 to complete the sulphonic reaction, as it will be found that no more sulphuric acid will combine organically even if the procedure is kept on longer. Whilst agitation and cooling are con- 15 tinued, one hundred twenty parts of refined mineral oil with a specific weight of about .800 to .820 are added at once to the sulphonated oil. It is not necessary to wash the sulphonated oil for the purpose of eliminating any excess of uncom- 20 bined sulphuric acid before adding the mineral oil as, instead of being a hindrance, presence of said excess sulphuric acid is necessary in order to produce the improved composition of sulphonated oil and mineral oil or other hydrocarbon, 25 which mixture has the properties described and is homogeneous and transparent. Agitation during ten more minutes will bring about the desired homogeneity of the compound, after which the excess sulphuric acid is substantially removed 30 by means, e. g., of sodium hydroxide in the form of lye of about 16° Bé. until the pH value is between 7 and 9. The lye is added in a thin stream (whilst stirring and cooling continue uninterrupted) until the compound turns to a yellow- 35 brown color. At this moment, a small quantity placed in a test tube will show it to be clear. Upon mixing the resulting product with water it will go at once into solution and form an emulsion of high stability in which dispersion or subdivision reaches the point where the Brownian move- 40 ment can be detected.

2. Incorporate, under the effects of a powerful and rapidly moving mechanical agitator or mixer, five parts of benzol and five parts of naphthalene, 45 (both of ordinary commercial grade and purity), within an oil mixture obtained with ten parts of castor oil (oleum ricini), ten parts of liquid fatty acids of common tallow (oleic acid, red oil), twenty parts of herring oil with an iodine number ranging between 160 and 180, and fifty parts 50 of ordinary sardine oil. Once the benzol and the naphthalene are completely dissolved in this mixture, incorporate five to eight parts of completely dried and finely pulverized acid sulphate of 55 potash. The mixture should be cooled down to +5° C. After thorough incorporation of this catalyst, sulphonation is brought about by adding thirty parts of concentrated sulphuric acid. As in the previous formula, one half of the quantity of this sulphuric acid, i. e., fifteen parts, can 60 be poured at once into the vat. The temperature should not rise above 30° C. and, after about 20 minutes, should be down again to the initial +5° C. if stirring and cooling were properly conducted.

The remaining fifteen parts of sulphuric acid are then added, not all at once, but in the form of a thin stream so that the temperature will not rise above 30° C. After one full hour from the time the operation was started, the sulphonic reaction 5 is completed. Similarly as with the first formula, from two hundred sixty to three hundred parts of refined mineral oil with a specific weight of about .800, are now added all at once. Agitation during ten more minutes will bring about 10 the desired homogeneity, after which neutralization is performed as in the first formula. Upon mixing with water the resulting product, it will go at once into solution and form an emulsion of high stability, in which dispersion or subdivision 15 reaches the point where the Brownian movement can be detected. This product has eminent solutive, emulsive, dispersive, penetrating, lubricating, softening, and color enhancing properties, and carries with it into emulsion or dispersion 20 any other oils or greases added thereto. The properties with which it is endowed make it especially useful in the textile, tanning and dyeing industries.

What is claimed as new is:

1. In the sulphonation of oils and greases containing oleaginous material, the step comprising sulphonating the oleaginous material in the presence of an acid sulphate of an alkali metal at a rate to limit the temperature rise to approxi- 30 mately 30° C.

2. In the sulphonation of oils and greases containing oleaginous material, the step comprising sulphonating the oleaginous material with sulphuric acid in the presence of acid potassium 35 sulphate at a rate to limit the temperature rise to approximately 30° C.

3. In the sulphonation of oils and greases containing oleaginous material, the steps comprising sulphonating the oleaginous material with 40 an excess of sulphuric acid in the presence of an acid sulphate of an alkali metal at a rate to limit the temperature rise to approximately 30° C., adding and mixing a hydrocarbon and then substantially eliminating the excess sulphuric acid. 45

4. In the sulphonation of oils and greases containing oleaginous material, the steps comprising sulphonating the oleaginous material with an excess of sulphuric acid in the presence of an acid sulphate of an alkali metal at a rate to limit 50 the temperature rise to approximately 30° C., adding and mixing a hydrocarbon and then adding an alkali until the pH value is from 7 to 9.

5. In the sulphonation of oils and greases containing oleaginous material, the steps comprising sulphonating the oleaginous material with an excess of sulphuric acid in the presence of an acid sulphate of an alkali metal at a rate to limit 55 the temperature rise to approximately 30° C., adding and mixing a hydrocarbon and then substantially eliminating the excess sulphuric acid by neutralization.

ALEXANDER GRESSNER.